# EUROPEAN PATENT SPECIFICATION

(11) **EP 0 056 263 B1**
(45) Date of publication and mention of the grant of the patent: **07.08.1985**
(21) Application number: 82100102.1
(22) Date of filing: 08.01.1982
(51) Int. Cl.: D21C 9/02, D21D 1/40

(54) **A method for improving the washing of cellulose pulps produced from lignocellulosic material**
Verfahren zur Verbesserung des Waschens von Cellulosepulpen, hergestellt aus Lignocellulosematerial
Procédé pour améliorer le lavage de pâtes cellulosiques préparées en partant d'une matière lignocellulosique

(30) Priority: 14.01.1981 SE 8100179
(43) Date of publication of application: 21.07.1982
(73) Proprietor: MO OCH DOMSJÖ AKTIEBOLAG, S-891 91 Örnsköldsvik (SE)
(72) Inventor: Lindahl, Jonas Arne Ingvar, S-89200 Domsjö (SE)
(74) Representative: Barz, Peter, Dr.

## Description

The present invention relates to a method for washing cellulose pulps produced from lignocellulosic material more effectively than when applying known washing techniques, so as to improve the recovery of chemicals and combustible organic materials from the waste liquors. By cellulose pulp is meant primarily chemicals pulps, semi-chemical pulps and chemi-mechanical pulps produced from both softwood and hardwood.

In the chemical pulping of lignocellulosic material there is obtained a residue which contains inorganic chemicals and dissolved organic substances, said substances comprising mainly lignin and minor quantities of cellulose, together with extractive substances, such as resin. Undesirable residual material is washed away. The waste liquor and washing liquid obtained are evaporated and burned, normally so that the chemicals can be recovered. Thus, in order to facilitate recovery of the chemicals, a washing effluent having the highest possible dry solids content is constantly sought for, i.e. attempts are made to use the least possible amount of water during the washing process.

When producing cellulose pulps with a yield in excess of about 55%, the wood chips are normally mechanically defibrated to separate fibre form, prior to washing and/or screening the pulp. When screening the pulp, there is obtained a concentration of the non-defibrated wood residues, referred to as reject or tailings, which are normally defibrated in a separate stage to separate fibre form, and then returned to the pulp flow.

The pulp suspension obtained subsequent to delignifying the wood chips can be washed in accordance with a number of mutually differing methods known to the art. The oldest method is one in which the pulp suspension is washed in so-called diffusers, i.e. a displacement wash which is carried out batchwise in large vessels. In another method, which is common at present, the pulp suspension is washed on drum filters, normally in several stages. The number of drum filters may vary, although normally from three to four filters are used. In a further and more recent method, pulp is washed with the use of presses whereat greater volumes of liquid can be removed than when using filters, which results in a more effective recovery of chemicals and organic substances.

When applying the aforedescribed washing techniques, however, significant quantities of residual chemicals and undesirable organic substances are left in the pulp, which, when the pulp is to be subsequently bleached, results in an unnecessarily high consumption of bleaching chemicals, and causes an undesirably high quantity of substances harmful to the environment to be discharged to the surroundings. Further, an increase in the extent to which chemicals used in the cellulose processes can be recovered is also highly desirable, both from an economic and environmental aspect.

The present invention affords a solution to the aforementioned problems and makes possible an increase in the extent to which chemicals are recovered. Accordingly, the invention relates to a method for improving the washing of unbleached cellulose pulp when producing cellulose pulps from ligno-cellulosic material, by chemical delignification, in which the pulp suspension is washed in a plurality of stages while supplying water thereto, characterised in that the pulp, after having been partially washed so that at least 10% of the dry solids content of the cooking waste liquor is removed, is subjected between a pair of successive washing stages or between several successive washing stages to a mild mechanical working treatment in a device adapted for high-consistency treatment and provided with screws rotating relative to each other at an energy input of from 7 to 200 kWh per ton of bone-dry pulp.

It has also been found particularly suitable to increase the pulp dry solids content prior to the mild mechanical treatment process, to between 10% and 50%, preferably to between 14 and 40%, and suitably to between 20 and 35%. Upon completion of the mild mechanical treatment process, the pulp suspension is diluted to a pulp consistency of between 0.5 and 13%, in conjunction with mixing with wash liquid in the subsequent washing step. When the pulp is washed on filters, the most suitable pulp consistency lies between 0.5 and 6%, while washing-dewatering in, for example, a press is suitably performed at an input pulp consistency of between 2 and 13%.

The mild mechanical treatment process according to the invention can be carried out at all temperatures normally used in practice. However, a particularly suitable temperature range is 20°-110°C, while a preferred range is 35°-90°C.

By mild mechanical treatment is meant here a process in which pulp suspensions of the aforementioned dry solids contents are subjected to a repeated pressing, kneading and shearing treatment, whereat the input of electrical energy for carrying out said treatment is held within the range of 7 to 200 kWh per ton of bone-dry pulp, and preferably within the range of 10 to 100 kWh per ton of bone-dry pulp.

It has been found particularly suitable to effect the mild mechanical treatment process according to the invention in a screw-type defibrator of the kind comprising two rotatable, bladed screws which are arranged parallel to one another in a housing provided with an inlet and outlet, and which are in adjustable meshing engagement with one another, to provide the mild mechanical treatment of the material, as before described. Conveniently, the screw blades of the rotatable screws also exhibit concave portions at the periphery of at least some of the screw turns, to form teeth-like protrusions between said concave portions. Screw defibrators of the aforedescribed kind are sold by MoDoMekan AB under the registered trademark FROTAPULPER@.

The novel method according to the invention, in which the pulp suspension is mechanically treated in a mild fashion between two or more of the stages of a washing sequence, has been surprisingly found to provide a cleaner pulp and to result in higher chemical recovery, a lower discharge of impurities to the surroundings and a higher dry solids content of the effluent washing water than was previously the case, when applying conventional washing techniques.

Thus, the present invention affords the important advantage of enabling a purer pulp to be obtained. This is manifested, inter alia, by a considerable lowering of the extractive content of the pulp and its kappa number.

The advantages afforded by the method according to the invention also include the possibility of increasing the dry solids content of the liquor departing from the pulp-washing stage, i.e. the amount of organic materials contained by said liquor, and also the amount of inorganic chemicals contained thereby. This increases the fuel value of the washing liquid, representing a valuable saving on energy. Because more contaminants are brought to evaporation and burning, and a greater amount of chemicals are recovered, the amount of environmentally harmful substances contained in the effluent is less than would otherwise be the case, which is an important advantage, and also desirable from an environmental aspect. Consequently, the cost involved in the treatment and destruction of environmentally harmful substances in the effluent can be reduced when applying the invention.

A further advantageous and surprising effect afforded by the invention is that the consumption of bleaching chemicals, such as chlorine, chlorine dioxide, hypochlorite, hydrogen peroxide and oxygen gas is markedly reduced when bleaching the washed pulp.

Another surprising effect obtained by the inclusion of the mild mechanical treatment process according to the invention, is that the dewatering of the resultant pulp suspension is markedly improved, a fact which affords decisive advantages when further treating the pulp.

The advantages afforded by the method according to the invention are further illustrated by the examples shown in the description.

The Figure illustrates schematically a suitable embodiment of the method according to the invention applied in washing tests with birch sulphate pulp and chemi-mechanical spruce pulp in three stages, each of said stages being equipped with a press. In the tests there was installed between the first and second washing stages a screw defibrator of the kind sold under the trademark FROTAPULPER@.

The following examples set forth experiments carried out in accordance with a preferred embodiment of the described method, together with the results obtained.

In the following tests, which were carried out in parallel, birch sulphate pulp and chemi-mechanical spruce pulp were washed in three stages, partly in accordance with the invention, incorporating said mild mechanical treatment process between the first and second washing stages (Examples 1 and 2), and partly in accordance with conventional techniques (Controls 1 and 2), in which the pulp suspensions were not subjected to any form of mechanical treatment between the different stages of the washing sequence.

The process diagram illustrated in the Figure was utilized in all tests, and hence the reference numerals below refer to corresponding references in the Figure.

### Example 1

Unbleached and unwashed birch sulphate pulp was introduced through a line 1 into a tank 2, in which the pulp suspension was diluted with press waste liquor supplied through a line 22, until a pulp consistency of about 8% was obtained. The pulp suspension was passed from the tank 2 through a line 3 to a first washing stage comprising a press 4, in which the pulp suspension was thickened to a dry solids content of 33.3% and then passed through a line 5, to a screw feeder 6, arranged to feed the pulp suspension through a line 7 and a line 8 to a screw defibrator 10 provided with two rotating screws whose blades exhibited concaved portions and in which the pulp suspension was subjected to a mild mechanical treatment process, whereafter said suspension was passed to a second screw feeder 12 through a line 11. The temperature of the pulp suspension at the inlet to the screw defibrator 10 was measured as 68°C, and at the outlet of said defibrator as 71°C. The amount of electrical energy consumed by the mild mechanical treatment process in the screw defibrator 10 was measured to 15 kWh per ton of bone-dry pulp. The line 9 was closed while passing the pulp suspension through the defibrator 10.

The treated pulp suspension was diluted in the screw feeder 12 to a pulp consistency of 8%, by introducing press waste liquor to said feeder through a line 21, said waste liquor mixing effectively with the pulp suspension during its transport through the feeder 12. The diluted pulp suspension was then passed through a line 13 to a second washing stage equipped with a press 14, comprising a press similar to that used in the first washing stage. The pulp suspension was washed and again thickened in the press 14, to a dry solids content of 33.3%. Waste liquor obtained from the press 14 was passed through a line 22 to the tank 2, where it was used to dilute incoming pulp suspension. The pulp suspension, washed and thickened in the second washing stage, was then passed through a line 15 to a screw feeder 16, and through a line 17 to a third washing stage equipped with a press 18 similar to the presses used in the two preceding washing stages.

The pulp suspension was diluted and mixed in the screw feeder 16 in a manner similar to that in the preceding screw feeder 12, although in this case with pure water supplied through a line 20, to obtain a pulp consistency of 8%. Subsequent to washing the pulp suspension and thickening the same to a dry solids content of 33.3% in the press 18, the finally washed pulp suspension was removed through a line 19.

Press waste liquors were removed from the lines 21 and 22 during the tests, for analysis purposes. Samples of the finally washed pulp were also taken from the line 19. The analysis results are shown in Table 1. Waste liquor from the press in the first washing stage 4 was taken through a line 23 and passed to a recovery plant (not shown in the drawing), where said waste liquor was evaporated and burned. Because the washing liquid was passed in counter-flow to the flow of pulp suspension, and because of the mechanical treatment to which the pulp suspension was subjected, the press waste liquor had a high organic-substance content (about 13%) and, at the same time, a high fuel value.

### Control test 1

In this test there was washed a birch sulphate pulp taken from the same batch as the pulp used in Example 1 and treated in the same apparatus, although with the difference that the pulp suspension was not subjected to a mild mechanical treatment process between the first and second washing stages. Thus, all flow of pulp suspension through the line 8 was stopped, so that the pulp suspension passed instead directly to the second screw feeder 12, through the line 9.

Subsequent to washing and thickening the pulp suspension in the press 14 of the second washing stage, there was obtained in this case a dry solids content of 26%. After washing and thickening the suspension in the press 18 of the third washing stage, there was also obtained a dry solids content of 26%. It will be noted that the consistency of the pulp suspension at the inlets to presses 14 and 18 respectively was also 8% in this test, and that the pressure exerted by the presses was the same as that in Example 1.

Analysis samples were removed in this test at the same locations as in the test according to Example 1. The analysis results are shown in Table 1 below.

As will be seen from the Table, when applying the method according to the invention quite surprisingly a considerably better washing was obtained than can be obtained when washing in accordance with known techniques. Thus, for example, despite the fact that the mild mechanical treatment process was carried out on a pulp suspension which had only been partially washed, the method according to the invention surprisingly resulted in a pulp with a much lower extractives content than can be obtained when conventionally washing pulp without mechanically treating the pulp between washing stages.

One important advantage with respect to energy afforded by the increased extent to which organic substances are washed from the pulp is that the fuel value of the waste liquor is also increased. Further a higher percentage of the cooking chemicals are recovered.

### Example 2

The test described in Example 1 was repeated with chemi-mechanical spruce pulp cooked to a pulp yield of 73%, calculated on absolute dry wood. After washing the pulp suspension and thickening the same in the press 14 of the second washing stage, there was obtained in this test a dry solids content of 34%. A dry solids content of 34% was similarly obtained after washing and thickening the pulp in the press 18 of the third washing stage. The line 9 was closed when making this test.

### Control test 2

In this test a similar type of chemi-mechanical spruce pulp was washed, and treated in the same plant as that used in Example 2, although with the difference that the pulp suspension was not subjected to any form of mild mechanical treatment between any of the washing stages. Thus all flow of pulp suspension through the line 8 was stopped, so that the pulp suspension instead passed directly to the second screw feeder 12, through the line 9. Subsequent to passing the press 14 of the second washing stage, the dry solids content was found to be 30%. The dry solids content was also found to be 30% after passing the press 18 of the third washing stage.

When making a comparison between washing the pulp in accordance with known techniques and washing the pulp in accordance with the present invention, it can be concluded that more water is removed and more chemicals recovered when practicing the method according to the invention. This conclusion is based on the fact that the volume of waste liquor recovered when applying the present invention was greater, despite the fact that the consistencies of the pulp suspensions entering the presses, in both tests, were maintained constant at 7%. According to measurements taken, the washing water in Example 2 also contained slightly larger quantities of dry solids than the washing water in Control test 2. Thus, it can be established that the fuel values of the liquors obtained when applying the method according to the invention are higher than the fuel values of corresponding liquors obtained when washing chemi-mechanical pulp in accordance with conventional techniques.

## Claims

1. A method for improving the washing of unbleached cellulose pulp when producing cellulose pulps from ligno-cellulosic material, by chemical delignification, in which the pulp suspension is washed in a plurality of stages while supplying water thereto, characterised in that the pulp, after having been partially washed so that at least 10% of the dry solids content of the cooking waste liquor is removed, is subjected between a pair of successive washing stages or between several successive washing stages to a mild mechanical working treatment in a device adapted for high-consistency treatment and provided with screws rotating relative to each other at an energy input of from 7 to 200 kWh per ton of bone-dry pulp.

2. A method according to claim 1, characterised in that the mild mechanical treatment process is carried out at a pulp dry solids content of between 10 and 50%, preferably between 14 and 40%, and more preferably between 20 and 35%.

3. A method according to claims 1 to 2, characterised in that the electrical energy input to the mild mechanical treatment process is held within the range of 10 to 100 kWh/ton.

4. A method according to claims 1 to 3, characterised in that the mild mechanical treatment process is carried out in a screw defibrator of the kind comprising two rotatable, bladed screws which are arranged parallel to one another in a housing provided with an inlet and an outlet, and which engage in each other for mildly treating the material, and the screw blades of which exhibit concave portions on the periphery of at least some screw turns to form tooth-like protrusions between said concave portions.

## Patentansprüche

1. Verfahren zum Verbessern des Auswaschens von ungebleichtem Cellulosehalbstoff bei der Herstellung von Cellulosehalbstoffen aus Lignocellulosematerialien durch chemische Delignifizierung, wobei die Halbstoffsuspension in mehreren Stufen unter Wasserzufuhr gewaschen wird, dadurch gekennzeichnet, dass der Halbstoff nach teilweisem Auswaschen, so dass mindestens 10% des Trockenfeststoffgehalts der Kochablauge entfernt sind, zwischen einem Paar von aufeinanderfolgenden Waschstufen oder zwischen mehreren aufeinanderfolgenden Waschstufen einer milden mechanischen Bearbeitung in einer Vorrichtung, die zur Dickstoffbehandlung geeignet und mit relativ zueinander rotierenden Schrauben ausgerüstet ist, bei einer Leistungsaufnahme von 7 bis 200 kWh pro Tonne knochentrockenem Halbstoff unterzogen wird.

2. Verfahren nach Anspruch 1, dadurch gekennzeichnet, dass die milde mechanische Behandlung bei einem Trockenfeststoffgehalt des Halbstoffs zwischen 10 und 50%, vorzugsweise zwischen 14 und 40% und insbesondere zwischen 20 und 35% durchgeführt wird.

3. Verfahren nach Anspruch 1 bis 2, dadurch gekennzeichnet, dass die elektrische Leistungsaufnahme bei der milden mechanischen Behandlung im Bereich von 10 bis 100 kWh/Tonne gehalten wird.

4. Verfahren nach den Ansprüchen 1 bis 3, dadurch gekennzeichnet, dass die milde mechanische Bearbeitung in einem Schraubenzerfaserer des Typs durchgeführt wird, der zwei drehbare mit Blättern versehene Schrauben aufweist, die in einem mit einem Einlass und einem Auslass versehenen Gehäuse parallel zueinander angeordnet sind und zur milden Bearbeitung des Materials ineinander eingreifen und deren Schraubenblätter am Aussenumfang zumindest einiger Schraubenwindungen konkave Bereiche aufweisen, so dass zahnähnliche Vorsprünge zwischen den konkaven Bereichen ausgebildet werden.

## Revendications

1. Procédé pour améliorer le lavage de pâte cellulosique non blanchie lors de la fabrication de pâtes cellulosiques en partant de matière lignocellulosique par délignification chimique, procédé dans lequel on lave la suspension de pâte en plusieurs stades tout en y amenant de l'eau, caractérisé par le fait qu'après l'avoir lavée partiellement de façon qu'au moins 10% de la teneur en solides secs de la lessive résiduaire de cuisson soient éliminés, on soumet la pâte, entre deux stades successifs de lavage ou entre plusieurs stades successifs de lavage, à un traitement modéré de travail mécanique dans un appareil conçu pour le traitement à consistance élevée et muni de vis tournant l'une par rapport à l'autre, avec une fourniture d'énergie de 7 à 200 kWh par tonne de pâte absolument sèche.

2. Procédé selon la revendication 1, caractérisé par le fait que l'on effectue le processus de traitement mécanique modéré à une teneur en solides secs de la pâte comprise entre 10 et 50%, de préférence entre 14 et 40% et de préférence encore entre 20 et 35%.

3. Procédé selon l'une ou l'autre des revendications 1 ou 2, caractérisé par le fait que l'on maintient la fourniture d'énergie électrique au processus de traitement mécanique modéré dans la gamme de 10 à 100 kWh/t.

4. Procédé selon l'une quelconque des revendications 1 à 3, caractérisé par le fait que l'on conduit le processus de traitement mécanique modéré dans un défibreur à vis du genre comprenant deux vis à lames tournantes, qui sont disposées parallèlement l'une à l'autre dans une enveloppe munie d'une entrée et d'une sortie, qui s'engagent l'une dans l'autre pour traiter modérément la matière et dont les lames de vis présentent des parties concaves à la périphérie d'au moins certaines spires de vis pour former des saillies similaires à des dents entre les parties concaves.
